

## UNITED STATES PATENT OFFICE

2,026,614

PAVING COMPOSITION AND PROCESS OF  
PRODUCING SAME

Joseph H. Conzelman, Birmingham, Ala., assignor  
to Alabama Asphaltic Limestone Company, Bir-  
mingham, Ala., a corporation of Alabama

No Drawing. Application January 8, 1934,  
Serial No. 705,738

7 Claims. (Cl. 106—31)

This invention relates to cold laid rock asphalt pavements of the type in which asphalt derived from a water external asphalt emulsion is used as a flux and binding medium.

5 More particularly this invention relates to the preparation of a cold laid rock asphalt mixture that will be dense and low in voids when compacted, but still easily workable while being transported; one that will have properties that allow it 10 to readily bond together when compressed while still being stable after compression and subjected to traffic.

Many cold laid mixtures in which a liquefied asphalt is used as the binding medium are not 15 dense when compacted. The high void surfaces laid with such mixtures are very susceptible to deterioration due to action of the elements. They cannot be designed to provide fines for a closed, low void mixture, for if so designed a portion 20 of the volatile liquefier stays in the mixture and an unstable pavement results that will shove and wave under traffic.

This difficulty is overcome, to a large extent, when the aggregate, both coarse and fine, used 25 in these mixtures is crushed rock asphalt. Even with this material, which imparts extraordinary stability to any bituminous paving mixture, especially in the case of the limestone rock asphalts, there are combinations of conditions that make 30 a cold laid rock asphalt in which liquefied asphalt, or a liquefier and an asphalt cement are used, dangerous. Such mixtures when laid to a greater thickness or depth than usual on streets that have to be opened to traffic immediately, requiring 35 rolling of the mixture as soon as it is spread with no time allowed for evaporation of the volatile content, may make unstable surfaces, especially if the weather when the mixture is laid is cold. These are conditions that should 40 not exist on a well supervised job, but which nevertheless frequently prevail.

The mixture covered by this invention would be a safe one to lay under such conditions. It involves the use of a small, safe amount of a solvent 45 for bitumen such as naphtha, gasoline or in some instances kerosene to soften the hard asphalt with which the rock asphalt is impregnated. The purpose of the use of such solvent is not to make the resulting mixture workable and easy to 50 handle. In fact a sufficient amount for this purpose is not used. The solvent merely serves to soften the natural asphalt in the rock asphalt and to bring it to a condition or state that will make it more readily flux with the asphalt cement 55 in the asphalt emulsion used as a bonding and

fluxing medium in this mixture. The advantage of this lies in the ability of this emulsion mixture to bond together and acquire stability more quickly when so treated than would be possible if the character of the native asphalt in the rock asphalt was not changed. This native asphalt in most instances is very hard, seldom having a penetration of over 20 and the process of cold fluxing this asphalt with the relatively hard asphalt in a proper asphalt emulsion must 10 necessarily be slow and be accomplished after the mixture is laid in the pavement and subjected to traffic. During this period such a mixture would not have the bonding qualities or the stability of mixture treated as described in this invention. In the case of rock asphalt containing 15 softer native asphalt the use of a small percentage of solvent to further soften the native bitumen and facilitate fluxing with the asphalt in the emulsion would also be of value. 20

For the purpose of description of design and preparation of my mixture, I may introduce into a mixer a batch of crushed fragments of rock asphalt, such as asphaltic limestone ranging in size from one-half inch to dust and so graded as to result in a dense low void mixture. This batch of say 2,000 pounds, would be treated with from 5 to 10 pounds of naphtha or gasoline, (one-fourth to one-half percent by weight relative to the limestone), thoroughly mixed with the asphaltic limestone and slightly fluxing the natural hard asphaltic cement in the exposed pores of the particles of rock. The amount of solvent should, in no case, exceed 0.8% by weight, relative to the asphaltic limestone. 35

If necessary to make the asphalt emulsion mix uniformly through the batch, water in the amount of say from 5% to 10% by weight of asphaltic limestone may now be added and uniformly mixed. 40

A water external asphalt emulsion is now added in sufficient amount, which may be 20 gallons, and mixed continually until the emulsion is uniformly distributed. 45

In this example the rock asphalt considered is an asphaltic limestone containing from 4 to 6% of natural bitumen having a penetration at 77° F. in 100 gm., 5 seconds, 15 to 20. The emulsion used with this rock asphalt would be an asphalt in 50 water emulsion that when mixed in proportions of one-third Portland cement and two-thirds emulsion, will not break during a ten minute period of mixing. The asphalt cement contained in the emulsion should have a penetration from 120 to 55

200 at 77° F., for the particular rock asphalt used in this example.

I do not wish to be limited to any exact proportions, however, as these depend on factors that 5 vary for individual cases. The characteristics of the rock asphalt, its grading, time of year when mixture will be laid and character of traffic, are factors. Preferably, the total asphalt in the mixture as laid on the road comprises from about 10 7½% to about 10½%, by weight of the total mixture.

Crushed stone, slag, gravel or sand might be added to the mixture but preferably should not exceed 50% by weight of the asphaltic limestone 15 used.

It is possible under certain conditions, that the naphtha or other solvent for the natural asphalt in the asphaltic limestone would be effective if added to the mixture after first adding the asphalt 20 emulsion and it is not the intention to confine this mixture to the exact procedure outlined in the example. The above example will suffice to illustrate the invention to anyone familiar with the art.

25 It is also to be understood that water to mix and coat each particle of rock, may be dispensed with under certain conditions.

I claim as my invention:

1. The process of producing a cold laid paving mixture of the character described, which 30 comprises adding to crushed rock asphalt a volatile solvent for bitumen in an amount merely sufficient to soften the hard native asphalt in the rock asphalt and facilitate the fluxing of this 35 native asphalt with the asphalt in the bonding medium, adding an aqueous asphalt emulsion and agitating said materials in a mixture until a homogeneous mixture results.

2. The process of producing a cold laid paving 40 mixture of the character described, which comprises adding to crushed rock asphalt a volatile solvent for bitumen in an amount merely sufficient to soften the hard native asphalt in the rock asphalt and facilitate the fluxing of this 45 native asphalt with the asphalt in the bonding medium, adding sufficient water to moisten the crushed rock asphalt particles, adding an asphalt in water emulsion, and agitating the materials until a homogeneous mixture is formed.

50 3. The process of producing a cold laid paving mixture of the character described, which comprises adding to crushed rock asphalt less than 0.8% by weight of the rock asphalt of a

volatile solvent for bitumen which has the capacity of softening the hard native asphalt in the rock asphalt and facilitating the fluxing of this native asphalt with the asphalt in the bonding medium to be added, then adding a water external 5 asphalt emulsion and agitating said materials in admixture until a homogeneous mixture results.

4. The process of producing a cold laid paving mixture of the character described, which comprises adding to crushed rock asphalt less than 10 0.8% by weight of the rock asphalt of a volatile solvent for bitumen which has the capacity of softening the hard native asphalt in the rock asphalt and facilitating the fluxing of this native asphalt with the asphalt in the bonding medium 15 to be added, adding sufficient water to moisten the crushed rock asphalt, then adding a water external asphalt emulsion and agitating said materials in admixture until a homogeneous mixture results. 20

5. The process of producing a cold laid paving mixture of the character described, which comprises adding to crushed rock asphalt an aqueous asphalt emulsion, agitating the mixture to uniformly distribute the emulsion there- 25 through, then adding a volatile solvent for bitumen in an amount merely sufficient to soften the asphalt in the rock asphalt and facilitating the fluxing of this native asphalt with the asphalt in the asphalt emulsion, and continuing the mix- 30 ing operation until a homogeneous mixture results.

6. The process of producing a cold laid paving mixture of the character described, which comprises adding to crushed rock asphalt sufficient 35 water to moisten the crushed rock asphalt then adding an aqueous asphalt emulsion, agitating the mixture to uniformly distribute the emulsion therethrough, then adding a volatile solvent for bitumen in an amount merely sufficient to soften 40 the asphalt in the rock asphalt and facilitating the fluxing of this native asphalt with the asphalt in the asphalt emulsion, and continuing the mix- 45 ing operation until a homogeneous mixture results.

7. A paving mixture comprising a water coated crushed rock asphalt whose hard native asphalt has been softened by a volatile solvent for bitumen in an amount limited to that which can be quickly taken up by the hard native asphalt, said 50 solvent being less than 0.8% by weight of the rock asphalt, and an aqueous asphalt emulsion.

JOSEPH H. CONZELMAN.